# EUROPEAN PATENT SPECIFICATION

(11) **EP 0 877 786 B1**
(45) Date of publication and mention of the grant of the patent: **04.12.2002**
(21) Application number: 96933428.3
(22) Date of filing: 25.09.1996
(51) Int. Cl.: C11D 3/00, C11D 1/835

(54) **FABRIC SOFTENING COMPOSITION**
GEWEBEWEICHMACHERZUSAMMENSETZUNG
COMPOSITION ASSOUPLISSANTE POUR TEXTILES

(30) Priority: 23.10.1995 GB 9521667
(43) Date of publication of application: 18.11.1998
(62) Divisional of application: 01123909.2
(73) Proprietor: UNILEVER PLC, London EC4P 4BQ (GB); UNILEVER N.V., 3013 AL Rotterdam (NL)
(72) Inventor: TURNER, Graham, Andrew, Bromborough Wirral Merseyside L62 6DD (GB)
(74) Representative: Elliott, Peter William
(86) International application number: EP9604260
(87) International publication number: WO97015651

(56) References cited:
- EP-A- 0 409 504
- EP-A- 0 568 297
- WO-A-95/27777
- WO-A-97/08285
- WO-A-97/12952

## Description

### Field of the Invention

The present invention relates to a fabric softening composition, in particular the invention relates to aqueous dispersions of fabric softening compositions comprising a water insoluble quaternary ammonium material and a nonionic stabilising agent suitable as rinse-added fabric softener compositions.

### Background of the Invention

Rinse added fabric softeners are known. Typically such compositions contain a water insoluble quaternary ammonium fabric softening agent dispersed in water at a level of softening agent up to about 7 wt%, in which case the compositions are considered dilute, or at levels from 7 wt% to 50 wt%, in which case the compositions are known as concentrates.

The viscosity of fabric softener may be seen by the consumer as an important attribute. For this reason thickening polymers are added to compositions, for example EP 0 331 237 (Unilever) discloses the use of hydrophobically modified nonionic cellulose ether for use as a thickener for fabric conditioning compositions containing quaternary ammonium cations.

There are however negative attributes associated with many polymeric thickeners in that they are not biodegradable, their addition to the rinse product is technically difficult and the viscosity of such polymer thickened products tends to increase with time.

WO 97/08285 discloses fabric softening compositions based on a mixture of an tertiary amine and a quaternary diester fabric softener where at least about 20% of the hydrocarbon substituent groups present in the tertiary amine and the quaternary di-ester fabric softener are unsaturated.

WO 97/12952 discloses a detergent composition comprising an amphoteric and/or a nonionic surfactant together with a substantially water insoluble fabric softening compound, and a detergency booster. The amphoteric/nonionic surfactant solubilises the fabric softening compound.

In US 4 137 180 (Lever Brothers Company) discloses cationic di-esters of the formula wherein R₁, R₂ and R₃ are each an alkyl or hydroxyalkyl group containing from 1 to 4 carbon atoms, or a benzyl group, R₄ and R₅ are each alkyl chains containing from 11 to 23 carbon atoms and X⁻ is a water soluble anion.

One of the problems associated with fabric softening compositions containing cationic di-esters as disclosed in US 4 137 180 is the physical instability of these compounds, the problem is exacerbated at temperatures above or below ambient.

EP 280 550 and EP 507 478 (Unilever) discloses the use of selected nonionic stabilising agents to overcome the poor stability. However we have found that many nonionic stabilising agents create a further problem in that their presence destroys the viscosity of these fabric softening compositions.

EP 409 504 (Unilever ) discloses fabric softening compositions comprising at least 1% w/w of an ester linked quat and an extruder material which can be esters of predominantly linear C₈-C₂₈ fatty acids with polyhydric alcohols.

WO 95/27777 discloses rinse conditioners comprising a fabric softening compound and a solubilising agent to be coated onto a tumble dryer sheet.

We have now found that selected nonionic stabilising agents do not destroy the viscosity of fabric softening compositions containing a biodegradable quaternary ammonium material.

### Description of the Invention

Accordingly the present invention relates to a fabric softening composition comprising:

Accordingly the present invention relates to an aqueous fabric softening composition comprising:
a) An aqueous dispersion of a water insoluble, quaternary ammonium material comprising at least one ester link and two C₁₂₋₂₈ alkyl or alkenyl groups;
b) from 0.1 wt% to 2.5 wt% of the total composition of a nonionic stabilising agent which is a sucrose ester;
where the sucrose ester is a mixture of a mono-ester, di-ester and a tri-ester and 56 to 75 wt%, based on the total weight of sucrose ester, is a sucrose mono-ester.

Further disclosed is A process for making a liquid fabric softening composition comprising the steps of selecting the following ingredients:
a) a water insoluble, quaternary ammonium material comprising at least one ester link and two C₁₂₋₂₈ alkyl groups;
b) a nonionic stabilising agent which is a mixture of sucrose mono-ester, sucrose di-ester and sucrose tri-ester where 56 to 75wt% based upon the total weight of the sucrose ester is a sucrose mono-ester;
c) other optional ingredients;
then mixing the ingredients whilst heating to form a melt, followed by dispersing the melt in water, to form an aqueous dispersion of the water insoluble quaternary ammonium material, containing 0.1 wt% to 2.5 wt%, based on the total composition, of the nonionic stabilising agent.

### Detailed Description of the Invention

The present invention is a way of controlling the viscosity of a fabric conditioner composition containing a biodegradable quaternary ammonium material and a nonionic stabilising agent.

Without wishing to bound by theory, this invention is thought to operate in that the interaction of the hydrogen bonding elements of the molecules of the nonionic stabilising agent are essential to maintain a vesicular structure. A vesicular structure in the context of this invention can be defined as a spherical structure having onion ring shaped bilayers. The presence of such vesicular structures are an important factor in the formation of a composition with a commercially acceptable viscosity.

The preferred level of nonionic stabilising agent present is 0.1 to 2.5 % by weight.

Most preferred nonionic stabilising agents are the sucrose esters. The sucrose esters have the additional benefit that they impart additional softening benefits over the cationic softening agent. Examples of suitable sucrose esters include the Crodesta (Trademark (ex Croda)) series. Crodestas are sucrose esters esterified with 70/30 mixture of stearic/palmitic acid to form a mixes of mono-ester, di-ester and triester. According to the manufacturer the levels of mono-ester are as follows:

| **Trade Name** | **wt % monoester** |
|---|---|
| Crodesta F10 | 3 |
| Crodesta F20 | 10 |
| Crodesta F50 | 29 |
| Crodesta F70 | 56 |
| Crodesta F110 | 52 |
| Crodesta F140 | 57 |
| Crodesta F160 | 75 |

We have found that these combination of mono-esters and di-esters and triesters of sucrose give particularly good softening benefits. Especially preferred are combinations of mono-ester, di-ester and triester that contain 56-75% monoester, in particular Crodesta F160, Crodesta F140, Crodesta 110 and Crodesta F70.

The fabric softening compound is suitably a substantially water insoluble quaternary ammonium material comprising a polar head group and two alkyl or alkenyl chains each having an average chain length greater than or equal to C₁₄, and at least one ester group.

Preferably the fabric softening compound of the invention has two long chain alkyl or alkenyl chains, each having an average chain length greater than or equal to C₁₆. Most preferably at least 50% of each long chain alkyl or alkenyl group has a chain of C₁₈.

It is preferred if the long chain alkyl or alkenyl groups of the fabric softening compound are predominantly linear.

The fabric softening compounds used in the compositions of the invention are molecules which provide excellent softening, and characterised by a chain melting -Lβ to Lα - transition temperature greater than 25°C, preferably greater than 35°C, most preferably greater than 45°C. This Lβ to Lα transition can be measured by DSC as defined in "Handbook of Lipod Bilayers, D Marsh, CRS Press, Boca Raton Florida, 1990 (Pages 137 and 337).

Substantially insoluble fabric softening compounds in the context of this invention are defined as fabric softening compounds having a solubility less than 1 x 10⁻³ wt% in demineralised water at 20°C. Preferably the fabric softening compounds have a solubility less than 1 x 10⁻⁴. Most preferably the fabric softening compounds have a solubility at 20°C in demineralised water from 1 x 10⁻⁸ to 1 x 10⁻⁶.

It is especially preferred if the fabric softening compound is a water insoluble quaternary ammonium material which comprises a compound having two C₁₂₋₁₈ alkyl or alkenyl groups connected to the molecule via at least one ester link. It is more preferred if the quaternary ammonium material has two ester links present. An especially preferred ester-linked quaternary ammonium material for use in the invention can be represented by the formula: wherein each R1 group is independently selected from C₁₋₄ alkyl, hydroxyalkyl or C₂₋₄ alkenyl groups; and wherein each R² group is independently selected from C₈₋₂₈ alkyl or alkenyl groups; X⁻ is any suitable anion.

T is and
n is an integer from 0-5.

Di(tallowyloxyethyl) dimethyl ammonium chloride is especially preferred.

A second preferred type of quaternary ammonium material can be represented by the formula : wherein R¹,X⁻,n and R² are as defined above.

Preferred materials of this class such as 1,2 bis[hardened tallowoyloxy]-3- trimethylammonium propane chloride and their method of preparation are, for example, described in US 4 137 180 (Lever Brothers). Preferably these materials comprise small amounts of the corresponding monoester as described in US 4 137 180 for example 1-hardened tallow-oyloxy-2-hydroxy-3- trimethylammonium propane chloride.

It is preferred if the quaternary ammonium compound is biodegradable. Biodegradable in the context of this invention should be interpreted as meaning degrades to materials that are not known to be harmful to the environment.

The ratio of quaternary ammonium material to nonionic stabilising agent is in the range from 5:0.5 to 5:0.1.

The composition may also contain long chain fatty acid material for example C₈ - C₂₄ alkyl or alkenyl monocarboxylic acids or polymers thereof. Preferably saturated fatty acids are used, in particular hardened tallow C₁₆ - C₁₈ fatty acids. Preferably the fatty acid is non-saponified, more preferably the fatty acid is free for example oleic acid. lauric acid or tallow fatty acid.

The level of fatty acid material is preferably more than 0.1%, more preferably more than 0.2% by weight. Especially preferred are dilutes in which the fatty acid material is present from 0.25 wt% to 20 wt%. The weight ratio of quaternary ammonium compound to fatty acid material is preferably from 1:10 to 10:1.

It is desirable if the viscosities of these fabric compositions lie in the range from 15 mPa.s to 120 mPa.s at a shear rate of 110s⁻¹.

The compositions of the invention preferably have a pH of more than 2, more preferably between 2 and 5.

The composition can also contain one or more optional ingredients, selected from the group consisting of nonaqueous solvents, pH buffering agents, perfumes, perfume carriers, fluorescers, colorants, hydrotopes, antifoaming agents, antiredeposition agents, enzymes, optical brighteners, opacifiers, antishrinking agents, drape imparting agents, antistatic agents and ironing aids.

The composition may also contain nonionic fabric softening agents such as lanolin and derivatives thereof.

The invention will now be illustrated by the following nonlimiting examples.

### EXAMPLES

In the examples all percentages are expressed by weight.

Comparative examples are represented by a letter while examples of the invention are represented by a number.

In the Examples HEQ is 1,2 bis[hardened tallowoyloxy]-3-trimethylammonium propane chloride ex Hoechst.

### Preparation of Fabric Conditioning Composition

Liquid fabric softening agents were made up as follows:

The cationic fabric softening agent and/or fatty acid and/or nonionic stabilising agent where appropriate were premixed and heated together to form a clear melt. The molten mixture thus formed was added over a period of at least one minute to water at 70°C to 80°C with constant stirring to form a dispersion.

### Viscosity Measurements

Viscosity was measured using the Haake RV20 Rotoviscometer. Viscosity is quoted at a shear rate of 10s⁻¹. The Casson data are obtained by using the Casson relationship:${\text{τ}}^{\text{0.5}} {\text{=τ}}_{\text{0}}^{\text{0.5}} {\text{+η}}_{\text{∞}}^{\text{0.5}} \text{.} {\text{D}}^{\text{0.5}}$ Where:
- τ =: Shear Stress (Pa)
- τ₀ =: Yield Stress (Pa)
- η_{∞} =: Infinite shear rate viscosity (mPa.s)
- *D* =: Shear rate (s⁻¹)

The Casson data were generated using the Haake RV20 Rotoviscometer with a range of shear rates from 0-1000s⁻¹.

### Examples 1-2 Comparative Examples A-D

Compositions were prepared in which an aqueous dispersion of 5% 6:1 HEQ:fatty acid, 0.5% of the following nonionics were added:

**Table 1**

| **Example** | **Nonionic** |
|---|---|
| A | No nonionic |
| B | Genapol T-150 |
| C | Tween 80 |
| D | Tween 85 |
| 1 | Crodesta F50 |
| 2 | Crodesta F110 |

Genapol, Tween and Crodesta are trade marks.

The effect of nonionic type on viscosity of a dilute quaternary ammonium compound is shown in Table 2.

**Table 2**

| **Example** | **η**_{**110**}**(mPa.s)** | **η-(mPa.s)** | **Comments** |
|---|---|---|---|
| A | 66 | 14.2 | Vesicular |
| B | 26 | 4.6 | No vesicles |
| C | 15 | 5.4 | No vesicles |
| D | 16 | 8.4 | No vesicles |
| 1 | 87 | 22.0 | Vesicles |
| 2 | 48 | 12.3 | Vesicles |

It can be seen that in the absence of nonionic the composition has a vesicular structure and accordingly has an acceptable viscosity. However the presence of nonionics stabilising agents which are not as specified by this invention, such as Genapol T-150, Tween 80 and Tween 85, do not allow vesicle formation and hence the viscosity of the composition is unacceptably low. The examples according to the invention allow vesicle formation and so have an acceptably high viscosity.

### Comparative Examples E-G

Compositions were prepared in which 0.5% of the following nonionic were placed in a composition containing an aqueous dispersion of 5% 6:1 dihardened tallow dimethyl ammonium chloride:fatty acid.

| | |
|---|---|
| Example E | No nonionic |
| Example F | Genapol T-150 |
| Example G | Crodesta F50 |

The results are shown in Table 3.

**Table 3**

| **Example** | **η**_{**110**}**(mPa.s)** | **η**_{**-∞**}**(mPa.s)** | **Comments** |
|---|---|---|---|
| E | 184 | 21.8 | Vesicular |
| F | 238 | 10.9 | Vesicular |
| G | --- | ---- | Vesicular |

Table 3 demonstrates that nonionic stabilising agents do not destroy the viscosity in formulations containing dihardened tallow dimethyl ammonium chloride.

### Examples 3-10 Comparative Examples A-B

To a base formulation of 5% HEQ:Hardened tallow fatty acid 6:1 in water the following nonionic stabilising agents were added:

| | | |
|---|---|---|
| Example 3 | 0.25 % | Crodesta F160 |
| Example 4 | 0.50 % | Crodesta F160 |
| Example 5 | 0.50 % | Crodesta F10 |
| Example 6 | 0.50 % | Crodesta F20 |
| Example 7 | 0.50 % | Crodesta F50 |
| Example 8 | 0.50% | Crodesta F70 |
| Example 9 | 0.50% | Crodesta F110 |
| Example 10 | 0.50 % | Crodesta F160 |

The softening performance of the sugar esters are demonstrated by Table 4.

**Table 4**

| **Examples** | **Softening Score** | **Total Votes** |
|---|---|---|
| 3 | 0.8828 | 31 |
| 4 | 1.0750 | 37 |
| A | 0.0000 | 6 |
| B | 0.5862 | 22 |

95% significance is obtained with a difference (Δ) between products of 0.9041. 90% significance is obtained when Δ=0.7565. It is thus demonstrated that the sucrose esters exhibit a significant softening benefit.

Table 5 demonstrates the optimum level of mono-ester present to maximise the softening effect.

**Table 5**

| **Example** | **Softening Score** | **Votes** |
|---|---|---|
| 5 | 0.0000 | 17 |
| 6 | 0.1689 | 25 |
| 7 | 0.2136 | 27 |
| 8 | 0.9444 | 54 |
| 9 | 1.3931 | 71 |
| 10 | 0.7005 | 46 |

## Claims

1. An aqueous fabric softening composition comprising:
a) An aqueous dispersion of a water insoluble, quaternary ammonium material comprising at least one ester link and two C₁₂₋₂₈ alkyl or alkenyl groups;
b) from 0.1 wt% to 2.5 wt% of the total composition of a nonionic stabilising agent which is a sucrose ester;
where the sucrose ester is a mixture of a mono-ester, di-ester and a tri-ester and 56 to 75 wt%, based on the total weight of sucrose ester, is a sucrose mono-ester.

2. A fabric softening composition according to claim 1 in which the ratio of quaternary ammonium material to nonionic stabilising agent is in the range from 5:0.5 to 5:0.1.

3. A fabric softening composition according to any preceding claim in which the viscosity of the composition is in the range from 15mPa.s to 120mPa.s at a shear rate of 110s⁻¹.

4. A fabric softening composition according to any preceding claim in which the composition further comprises more than 0.1 wt% of a fatty acid material.

5. A fabric softening composition according to claim 4 in which the fatty acid material is present from 0.25 wt% to 20 wt%.

6. A process for making a liquid fabric softening composition comprising the steps of selecting the following ingredients:
a) a water insoluble, quaternary ammonium material comprising at least one ester link and two C₁₂₋₂₈ alkyl groups;
b) a nonionic stabilising agent which is a mixture of sucrose mono-ester, sucrose di-ester and sucrose tri-ester where 56 to 75wt% based upon the total weight of the sucrose ester is a sucrose mono-ester;
c) other optional ingredients;
then mixing the ingredients whilst heating to form a melt, followed by dispersing the melt in water, to form an aqueous dispersion of the water insoluble quaternary ammonium material, containing 0.1 wt% to 2.5 wt%, based on the total composition, of the nonionic stabilising agent.

## Patentansprüche

1. Wässerige textilweichmachende Zusammensetzung, umfassend:
a) eine wässerige Dispersion eines in Wasser unlöslichen quaternären Ammoniummaterials, umfassend mindestens eine Esterbindung und zwei C₁₂₋₂₈-Alkyl- oder -Alkenylgruppen;
b) 0,1 Gewichtsprozent bis 2,5 Gewichtsprozent der Gesamtzusammensetzung eines nicht-ionischen stabilisierenden Mittels, das einen Saccharoseester darstellt,
wobei der Saccharoseester ein Gemisch eines Monoesters, Diesters und eines Triesters ist, und 56 bis 75 Gewichtsprozent, bezogen auf das Gesamtgewicht an Saccharoseester, ein Saccharosemonoester ist.

2. Textilweichmachende Zusammensetzung nach Anspruch 1,
wobei das Verhältnis von quaternärem Ammoniummaterial zu nicht-ionischem stabilisierenden Mittel im Bereich von 5:0,5 bis 5:0,1 liegt.

3. Textilweichmachende Zusammensetzung nach einem vorangehenden Anspruch,
wobei die Viskosität der Zusammensetzung im Bereich von 15 mPa·s bis 120 mPa·s bei einer Scherrate von 110 s⁻¹ liegt.

4. Textilweichmachende Zusammensetzung nach einem vorangehenden Anspruch,
wobei die Zusammensetzung weiterhin mehr als 0,1 Gewichtsprozent eines Fettsäurematerials umfasst.

5. Textilweichmachende Zusammensetzung nach Anspruch 4,
wobei das Fettsäurematerial mit 0,25 Gewichtsprozent bis 20 Gewichtsprozent vorliegt.

6. Verfahren zur Herstellung einer flüssigen, textilweichmachenden Zusammensetzung, umfassend die Schritte der Auswahl der nachstehenden Bestandteile:
a) eines in Wasser unlöslichen quaternären Ammoniummaterials, umfassend mindestens eine Esterbindung und zwei C₁₂₋₂₈-Alkylgruppen;
b) eines nicht-ionischen stabilisierenden Mittels, das ein Gemisch von Saccharosemonoester, Saccharosediester und Saccharosetriester darstellt, worin 56 bis 75 Gewichtsprozent auf das Gesamtgewicht an Saccharoseester ein Saccharosemonoester ist;
c) anderer wahlweiser Bestandteile;
dann Vermischen der Bestandteile unter Erhitzen zur Bildung einer Schmelze, gefolgt von Dispergieren der Schmelze in Wasser unter Bildung einer wässerigen Dispersion des in Wasser unlöslichen quaternären Ammoniummaterials, das 0,1 Gewichtsprozent bis 2,5 Gewichtsprozent, bezogen auf die Gesamtzusammensetzung, des nicht-ionischen stabilisierenden Mittels enthält.

## Revendications

1. Composition assouplissante aqueuse pour textiles comprenant :
a) une dispersion aqueuse de matériau ammonium quaternaire non soluble dans l'eau comprenant au moins une liaison ester et deux groupes alkyles ou alkényles en C₁₂₋₂₈ ;
b) de 0,1 % en poids à 2,5 % en poids, sur la base de la composition totale, d'un agent de stabilisation non ionique qui est un ester de saccharose ;
dans laquelle l'ester de saccharose est un mélange d'un mono ester, d'un diester et d'un triester, et 56 à 75 % en poids, sur la base du poids total d'ester de saccharose, est un mono ester de saccharose.

2. Composition assouplissante pour textiles selon la revendication 1, dans laquelle le rapport entre le matériau ammonium quaternaire et l'agent de stabilisation non ionique est compris dans la gamme allant de 5 pour 0,5 à 5 pour 0,1.

3. Composition assouplissante pour textiles selon l'une quelconque des revendications précédentes dans laquelle la viscosité de la composition est comprise dans la gamme allant de 15 mPa.s à 120 mPa.s à un taux de cisaillement de 110s⁻¹.

4. Composition assouplissante pour textiles selon l'une quelconque des revendications précédentes, dans laquelle la composition comprend en outre plus de 0,1 % en poids d'un matériau d'acide gras.

5. Composition assouplissante pour textiles selon la revendication 4, dans laquelle le matériau d'acide gras est présent dans une quantité allant de 0,25 % en poids à 20 % en poids.

6. Procédé de fabrication d'une composition liquide assouplissante pour textiles comprenant les étapes consistant à sélectionner les ingrédients suivants :
a) un matériau ammonium quaternaire non soluble dans l'eau comprenant au moins une liaison ester et deux groupes alkyles en C₁₂₋₂₈;
b) un agent de stabilisation non ionique qui est un mélange de mono ester de saccharose, de diester de saccharose et de triester de saccharose, dans lequel 56 à 75 % en poids, sur la base du poids total de l'ester de saccharose, est un mono ester de saccharose ;
c) d'autres ingrédients optionnels ;
puis à mélanger les ingrédients tout en chauffant afin de former un mélange fondu, puis à disperser le mélange fondu dans de l'eau afin de former une dispersion aqueuse du matériau ammonium quaternaire non soluble dans l'eau, contenant de 0,1 % en poids à 2,5 % en poids, sur la base de la composition totale, de l'agent de stabilisation non ionique.
